

April 1, 1930.

R. HUNTER

1,752,796

COLLAR

Filed May 26, 1925

Fig. 6



Fig. 1



Fig. 2



Fig. 3



Fig. 4



Fig. 5



Inventor:  
Ralph Hunter  
by  
Beers, Fisher & Cushman  
New York, N.Y.

## UNITED STATES PATENT OFFICE

RALPH HUNTER, OF NEW YORK, N. Y., ASSIGNOR TO HALL, HARTWELL & CO. INC.,  
OF TROY, NEW YORK, A CORPORATION OF NEW YORK

## COLLAR

Application filed May 26, 1925. Serial No. 32,955.

The object of this invention is to construct a fold-over shirt collar which, while having all of the merits of a fully starched collar, namely crisp, glossy and dressy appearance, 5 polished and therefore sanitary, and dirt-resisting surface, shall nevertheless be very flexible and comfortable to the wearer and (a very practical value) shall withstand a large number of launderings without cracking 10 at the fold line, which in fully starched collars is the most vulnerable point.

In fold-over collars of standard construction, comprising a band made of two plies or blanks of moderately fine cotton or linen 15 cloth, with, usually, an interlining blank of more open weave, and a top or fold-over portion, similarly made of two assembled cloth-blanks, with or without an interlining blank, the edge of the collar top is inserted 20 between edge-turned plies of the band, and then stitched in place. When the collar is starched and ironed, the fold of the top is in the collar top close to and parallel with the line of junction of top and band. As it is 25 along this fold line that collar fabric is ruptured after a few launderings, greater durability of the collar as a whole will be secured if the collar top be so constructed that its outer fabric will not be subjected to the 30 stresses, localized at the fold line, which produce fracture in fully starched collars as heretofore constructed.

The fold of the collar top, produced when the starched collar is ironed, and as the 35 starch material in it is heated or baked into solidity by the iron, involves tensile stress on the outer ply, and compressive stress on the inner ply. When, as has been the case in fully starched collars, the inner ply is saturated 40 with starch to the extent usual in laundry operations and this is baked into substantial solidity, it resists compression at the fold and thus enhances the tensile stress in the outer ply, which, also carrying a full 45 normal load of starch, subjects the individual yarns and their fibres to aggravated local tensile stresses, which after a few laundering operations result in fracture of the outer 50 ply along the fold line.

My improved collar is characterized by a

fold-over or top portion in which the outer ply is composed of a single-weave fabric so densely woven that its maximum starch-absorption capacity is substantially less than that of fabrics ordinarily used for the same 55 purpose and in the same part of a collar. The inner ply may be, but is not necessarily, made of fabric equally resistant to starch absorption. The quality of starch-exclusion or absorption-resistance, of the outer ply, not only reduces the percentage of starch that 60 will be absorbed into that ply, but to a substantial extent reduces the percentage of starch absorbed by the inner ply, which on its side adjacent to the outer ply is guarded against intrusion of starch. Thus the inner 65 ply of the collar top is softer and more yielding than as in starched collars as heretofore manufactured.

When, therefore, a collar provided with a 70 top portion constructed as above described, is ironed after having been immersed in the usual normal laundry solution of starch for the usual time and under the usual conditions of mechanical manipulation, the tensile stress 75 produced in the outer ply at the fold line is relieved by the local yielding of the inner 80 ply under compressive stress, and the yarns and fibres of the outer ply do not have to sustain stresses nearly as severe as those developed in the outer ply of the starched collar of the usual construction.

The same holds true if the top portion of a 85 collar comprising a starch absorption resisting outer ply is made with an open fabric interlining between the outer and inner plies.

If a collar top be made with its outer and inner ply both of absorption-resistant fabric, they mutually protect each other, reduce the starch content at and near their juxtaposed 90 surfaces, and provide the means, above described, for relieving the outer ply of fibre and yarn strains at the fold line.

To provide a cotton fabric so inherently 95 resistant to starch absorption that it will receive and retain, even after relaundering, as its usually and normally received starch content a percentage by weight materially less than that absorbable, and inevitably absorbed under similar normal laundry manipulation, by 100

ordinary collar fabrics, fine, long staple yarns are required. Preferably the warp yarns should be single ply, the filling yarns two ply, hard twisted.

5 The preferred weave-specifications (having in view a presentable cloth-texture) are 120 warp threads and 84 filling threads to the inch, or thereabouts. Good results in practice have been obtained, however, by varying the 10 relation of warp to filling, using 96 warps and 100 filling, per inch. In any case, and whatever the variations in pick and sley, the filling should be hard-beaten at the fell, so as to close the interstitial voids between yarns as 15 completely as possible. The count, or diameter, of both warp and filling yarns, while subject to some variation and choice, will be such as to combine, in the woven cloth, the aforesaid characteristics of high pick and sley, and 20 close texture, in a single weave cloth. Single cloth, as distinguished from double or other compound weaves, provides the characteristic of that thinness which is essential to high flexibility.

25 In the drawings hereto annexed, which illustrate my invention,

Fig. 1 is a section of outer ply collar top cloth, taken across filling and parallel with warp;

30 Fig. 2 is a section of the same, taken across warp and parallel with filling;

Fig. 3 is a section across warp and parallel with filling of cloth suitable for the inner ply of a collar top;

35 Fig. 4 is a section on a scale smaller than that of Figs. 1 to 3 inclusive, showing the relative weaves and thicknesses of outer ply and inner ply;

Fig. 5 is a vertical cross section of a fold 40 collar, taken on line 5—5 of Fig. 6; and

Fig. 6 is a plan view of a fold collar, opened or unfolded, exhibiting the outer plies of the collar top and collar band.

45 The effect of high pick and sley, and close weave and hard beat at the fell is indicated in Figs. 1 and 2. Where warp W and fillings F cross, they crush into each other, reducing the capillary voids in the fabric to a minimum, leaving practically no channels for ready infiltration of liquid starch solution. To some extent a starch solution penetrates between fibres of each yarn, but only a little into fine and hard twisted yarn, so that this slight 55 interfibre penetration and the indentations characteristic of the "tooth" of the fabric afford the only anchorage for a starch film. When a ply of such cloth is laid against a ply of the same or other cloth the penetration of 60 starch solution to the juxtaposed cloth surfaces is materially reduced.

For economy of manufacture a cheaper and less densely woven fabric may be used for the inner ply of the collar top, such as indicated 65 in Fig. 3. For instance, cotton cloth 72 warp

and 76 filling per inch will serve satisfactorily.

It is highly desirable, if not quite essential, that the outer or face fabric of the collar top be a single and simple "one and one" weave, 70 since this lends itself better than other weaves, twills for instance, to the dense and uniform absorption-resisting structure.

The usual structural assemblage of collar top T and band B is shown in Fig. 5. As indicated in Fig. 6, the flexibility of the collar as a whole may be enhanced by cutting sections of the outer ply of the collar band away, as at d. Since the collar band is never subjected to sharp folding, like the collar top, 80 it may be made of the usual qualities of fabric.

A collar top, made as above described, of 120 x 84 fabric in the outer ply and a fabric, plain weave, 72 x 76, when saturated to its 85 maximum absorbable content of starch, will absorb only about 14.5% by weight, of starch. Under the same conditions of immersion and maximum saturation the absorption-resistant outer ply cloth absorbs as its maximum 90 content about 13.5% of starch, whereas the inner ply cloth, 72 x 76 will absorb about 25%. This illustrates the protective effect of the 95 resistant outer ply material upon the more absorbent inner ply material, which manifests itself in similar manner under conditions of normal and usual laundry treatment which does not involve saturation of collar cloth to its maximum receptivity for the starch solution.

A fold collar, constructed on specifications like the foregoing has under test withstood thirty-five launderings without cracking, whereas full-starched collars as heretofore constructed all cracked in twelve launderings or less. The maximum absorbable content of starch, in the above recommended outer ply top-fabric is not more than 40% of the maximum absorbable by standard outer ply top-fabrics heretofore used. A 110 fabric capable of maximum absorption materially less than twenty per centum of its own weight of normal laundry starch solution, used in the outer ply of a fold-collar top produces under normal laundry treatment 115 substantially the above described results, even when assembled with a more absorptive inner ply.

Moreover, a collar constructed as above described, though the band be of ordinary 120 or standard specifications, is highly flexible even when starched with the starch solution and under the treatment usually employed in laundries for finishing the standard fully starched collars, capable of being wound 125 tightly around one's finger with no difficulty and with no injury to its finish or appearance when released. It therefore supplies the prevalent demand for a soft-feeling and comfortable collar, while it responds to the 130

demands of the most fastidious wearer in respect to "dressy" appearance. Unlike soft and "semi-soft" collars, it is light and smooth and agreeable to the touch, and has all the sanitary and soil-resisting properties of the fully starched and polished collar. It is, in truth, a fully starched collar, since it receives and retains all the starch it is capable of absorbing when treated with the normal starch solutions and in the same manner as has been the practice in laundries generally for the collars universally termed fully starched. At its surface there is present all the starch needed to receive as high a gloss as any collar should a glossy laundry finish be desired.

I claim:

1. A fold-collar comprising an outer top ply of single-ply weave of close texture and capable of maximum absorption materially less than twenty per centum of its own weight of normal laundry starch solution.
2. A fold-collar comprising in its top an outer ply of single-ply weave of close texture and capable of maximum absorption materially less than twenty per centum of its own weight of normal laundry starch solution and an inner ply protected by the outer ply against penetration of starch solution to the surface juxtaposed to said outer ply.
3. A fold-collar comprising in its top an outer ply of single-ply weave of yarns crushed together in the mesh to reduce the interstitial voids in the fabric to such degree of resistance to starch absorption that the said ply is capable of maximum absorption materially less than twenty per centum of its own weight of normal laundry starch solution.
4. A fold-collar comprising in its top an outer ply of single-ply weave of yarns crushed together in the mesh to reduce the interstitial voids in the fabric to such degree of resistance to starch absorption that the said ply is capable of maximum absorption materially less than twenty per centum of its own weight of normal laundry starch solution, and an inner ply of normally woven texture protected by said outer ply against penetration of starch solution to the surface juxtaposed to said outer ply.

Signed by me at Troy, New York, this 14th day of May, 1925.

RALPH HUNTER.